

Jan. 8, 1924.

1,479,865

H. G. METCALF

ROPE STRUCTURE

Filed June 18, 1923



Fig. 1



Fig. 2



Fig. 3

Inventor  
Harold G. Metcalf  
By *Clint & Cheney*  
his attorneys

## UNITED STATES PATENT OFFICE.

HAROLD G. METCALF, OF AUBURN, NEW YORK.

## ROPE STRUCTURE.

Application filed June 18, 1923. Serial No. 646,183.

*To all whom it may concern:*

Be it known that I, HAROLD G. METCALF, a citizen of the United States, residing at Auburn, in the county of Cayuga and State 5 of New York, have invented a certain new and Improved Rope Structure; and I do hereby declare the following to be a full, clear, and exact description of the same, reference being had to the accompanying 10 drawings, forming part of this specification.

This invention relates to improvements in cordage, particularly applicable to rope structures generally, that is to say, those 15 structures made up of three, four, six, or nine strands or readies assembled either in regular laid rope, or in cable-laid rope, the object of the invention being to increase the strength of the rope as well as the last- 20 ing qualities in the performance of work requiring constant bending or flexure, as well as in work wherein the rope is subjected to abrasion.

In the production of rope embodying the 25 present invention certain developments made in connection with the arrangement of the fibers in the rope structure are utilized with the object first of simplifying and reducing the cost of manufacture and, 30 secondly, of not only increasing the strength of the rope, under tension, but also increasing its flexibility and internal wear resisting qualities.

In accordance with the present invention, 35 the strands or readies from which the rope structure is built up are each composed of an internal portion wherein the main strength of the rope to resist tension strains is found, and an external portion designed 40 to resist wear and abrasion, but, of course, to a certain extent also adding to the tensile strength of the rope. The internal portion of each strand or ready is formed directly of sliver fibers and the fibers oc- 45 cupy substantially parallel relation to each other and are twisted only to a slight degree, usually conforming to the "forming" twist of the strand or ready, but the degree of twist may be varied in accordance with 50 known practice. Buried within the central sliver fiber portion of the strand or ready and preferably axially thereof, there is a

yarn or a ply yarn which yarn or ply yarn is thoroughly covered and impregnated with graphite or grease or water-proofing material having water repellent and lubricating qualities. Around the central portion of the rope strand or ready so formed of sliver fiber, there is wound in parallelism a covering composed of yarns or ply yarns and there may be one or a plurality of layers of such yarns or ply yarns to give the desired abrasive resisting qualities to the rope, as well as to exert a binding action on the central portion, in order to increase the strength of the rope by eliminating any tendency of the fibers to slip and separate from each other when subjected to severe tension strains, especially where the twist imparted to the sliver center is not in itself sufficient to accomplish this result. In some instances each of a series of slivers has incorporated in it a single yarn or a ply yarn which is thoroughly covered and impregnated with the lubricating and water resisting material or the lubricating yarn may be at the center and surrounded by the series of slivers, but in all cases it is embedded in a relatively large mass of sliver fiber.

In order that the use of the terms "sliver," "yarn," and "ply yarn" may be understood herein, such terms may be defined as follows: A "sliver" is a relatively large body of fibers which have been straightened and doubled the requisite number of times to insure uniformity and parallelism of the fibers, and this sliver fiber is in the rope structure, twisted only sufficiently to hold the fibers together and to prevent them from separating readily by being pulled apart. In some instances this sliver may have its individual fibers held together in part or in whole by the enclosing sheath of yarn or ply yarn. A "single yarn" is a relatively small body of fibers suitably doubled and straightened and twisted or spun into a structure, which has the relatively hard twisted characteristics of a thread or cord. A "ply yarn" is a plurality of single yarns which are twisted together and maintain their form or the characteristics of a cord formed of a plurality of single threads or yarns.

In the drawings:

Figure 1 represents a section of a three strand rope, one strand at the end being opened out to illustrate the internal structure;

Fig. 2 is a cross section of the rope illustrated in Fig. 1; and

Fig. 3 is a cross section illustrating a modification wherein a plurality of slivers 70 constitute the center portion of the rope and in each sliver there is embedded a lubricant impregnated single yarn or ply yarn.

Referring particularly to Figs. 1 and 2, the letter A indicates the enveloping sheath 15 for each of the strands or readies, this enveloping sheath being formed of a single or plural layers of yarns a. These yarns may be, as ordinarily, either single or ply yarns, but are preferably single yarns, inasmuch 20 as it is desirable to have the fibers of the yarns twisted together only to that degree which is necessary to constitute a good wearing or abrasion resisting cover or sheath, and at the same time to leave the fibers as free 25 as possible from all tendency to cut each other or to shear under the action of bending or tension stresses. The center portion of each strand or ready is formed of sliver fiber, a sliver or series of slivers preferably, 30 though not necessarily, four or more in number, as indicated at B, and these slivers have a twist imparted to them, which, in the preferred structure, substantially corresponds to the twist imparted to the whole ready or 35 strand in laying the sheath or cover thereon, in the rope machine, to which machine the sliver is preferably fed in a substantially untwisted condition. Embedded in the sliver fiber center so formed is the impregnated 40 yarn or ply yarn C which is illustrated in the drawings as a black center, indicating that it is impregnated with graphite, grease or other lubricating and water-proofing compound.

45 Instead of incorporating the lubricating yarn or ply yarn B in the center or along the axial line of each strand or ready, each of the slivers incorporated in the center may have an impregnated yarn E incorporated 50 therein, as indicated in Fig. 3 of the drawing, there being thus incorporated in each ready a plurality of impregnated yarns separated from each other by the fiber constituting the adjacent portions of the slivers from 55 which the center is formed, thus distributing the lubricating and water-repellant material throughout a greater area of the fiber.

The impregnated yarns so incorporated in the slivers are twisted to a greater degree 60 than the slivers themselves, and consequently present a greater length of fiber in a given length of rope. In other words, this yarn being a hard twisted portion of the structure will be capable of lengthening out when 65 stretched or elongation of the rope takes

place under tension strain or bending stress and will yet preserve its hard center lubricating quality.

By locating the lubricating impregnated 70 yarn in a surrounding body of soft fibers, so to speak, it is found that the distribution of the lubricant is not only such that it is most effective where lubrication is secured, but in use, the lubricant distributes itself 75 to the surrounding fibers and after a brief interval of use the center of the rope has lubricating qualities imparted thereto to a greater or less degree throughout, and from the beginning the rope as a whole is flexible to a degree which is practically impossible 80 of attainment in ropes heretofore produced and which were made of yarns in the ordinary way.

An additional advantage has become manifest in ropes of this character, due to the 85 fact that while the fibers constituting the rope are effectually clamped together, so to speak, as to prevent slipping with relation to each other, their entire tensile strength becomes available without that tendency to shear and cut, as in all hard laid ropes heretofore made, with the result that the tensile strength of a rope made in accordance with the present invention, as well as its capacity 90 for resisting bending stresses and constant 95 usage in bending or external abrasion are greatly increased.

It will be understood, of course, that the strands or readies may be laid together in 100 any ordinary way to form a rope, or a plurality of such ropes may be laid together in the ordinary way to form a cable. In other words, the strands may each form one-third of a regular laid rope, as illustrated in 105 the drawings, or they may form one-fourth or one-sixth of customary regular laid rope or one-ninth of cable laid rope, the latter being simply a structure made up of three regular laid ropes, as is well understood in 110 this art.

What I claim is:

1. A rope structure comprising a plurality of strands or readies laid together in twisted relation to form the finished rope, each of said strands comprising a twisted 115 yarn or ply yarn impregnated with a lubricating or water repellent substance and embedded in and surrounded by a relatively large body of sliver fibers twisted to a degree less than that of the impregnated yarn to form a relatively soft center, the whole being surrounded by yarns each twisted to a greater degree than the slivers, said yarns being spirally laid about the center and with adjacent yarns in contact with each other 120 to form an enveloping sheath.

2. A rope structure comprising a plurality of strands or readies laid together in twisted relation to form the finished rope, each of said strands comprising an envelope or 125

sheath of individually twisted yarns spirally laid about a center with adjacent yarns in contact, a relatively large sliver fiber center twisted to substantially conform to the spiral 5 lay of the enveloping yarns and a yarn or ply yarn of twisted fibers impregnated with lubricant embedded in the sliver center.

3. A rope structure comprising a plurality of strands or readies laid together in twisted 10 relation to form the finished rope, each of

said strands comprising an envelope or sheath of individually twisted yarns spirally laid about a center with adjacent yarns in contact, a relatively large center formed of a plurality of slivers twisted to conform 15 to the spiral lay of the enveloping yarns and a yarn or ply yarn of twisted fibers impregnated with lubricant and located centrally between the slivers.

HAROLD G. METCALF.